

May 19, 1931.

R. OMOTO

1,805,592

BLACK LINE PHOTOGRAPHIC SENSITIZED PAPER AND PROCESS OF MAKING THE SAME

Original Filed Jan. 25, 1928



INVENTOR:  
*R. Omoto*  
BY: *Marks & Clark*  
ATTORNEYS.

## UNITED STATES PATENT OFFICE

RYO OMOTO, OF TOKYO-FU, JAPAN, ASSIGNOR OF ONE-HALF TO MANABU TADA, OF TOKYO, JAPAN

## BLACK LINE PHOTOGRAPHIC SENSITIZED PAPER AND PROCESS OF MAKING THE SAME

Application filed January 25, 1928, Serial No. 249,504, and in Japan February 9, 1927. Renewed March 27, 1931.

This invention relates to a black line photographic printing paper adapted to give a print of black lines on a white surface when printed by artificial light or day light and it comprises a paper having a base coating of a plurality of soluble ferric salts, over which is disposed a coating of tannic acid or the like.

The chief object of my invention is to provide a paper yielding black lines on a white surface after exposure and immersion in water in much the same manner as ordinarily blue-print papers are manipulated. In my invention, I furthermore provide means whereby the operator can easily tell when exposure of the paper is completed.

In the process of making my paper, I first coat paper with a solution containing a plurality of ferric salts, a sulpho-cyanide and tartaric acid.

In manufacturing the paper, the liquid for the first coating is applied to a thin tenacious sheet such as the Japan Simili parchment paper, and the so treated paper is then dried. The constituents of the liquid and their relative quantities are not to be arbitrarily determined, but may be suited to various requirements. An example of the mixture is as follows:

|                         | Grams |
|-------------------------|-------|
| Ferric sulphate         | 2     |
| Ferric chloride         | 3     |
| Tartaric acid           | 2     |
| Gelatine                | 2     |
| Ammonium sulpho-cyanide | 1     |
| Distilled water         | 30    |

Then a solution of tannic acid or similar substances in a volatile solvent is applied to the paper coated with the ferric salt solution. The components of this solution and their corresponding percentage are not fixed, but meet the requisites on the occasion. An example is as follows:

|             |          |
|-------------|----------|
| Ether       | 80 c. c. |
| Alcohol     | 20 c. c. |
| Tannic Acid | 15 gms.  |

This second coating dries readily in a current of air in a few minutes. This completes the preparation of the paper.

The essentials of this invention, as already stated above, reside in mixing a sulpho-cyanide salt with the ferric salt solution and in using volatile liquids in which the tannic acid or similar matters are dissolved.

The reason why the two ferric salts are mixed together may easily be explained by the fact that the resulting black coloration of lines are distinctive, while the sole application of each single ferric salt produces only light black color. The tartaric acid sensitizes the ferric salts, which change to ferrous salts, when they are exposed to sunshine or intense electric light. These ferrous salts are not influenced by the tannic acid. The gelatine serves as an adhesive to bind the paper and the mixture, while it prevents the liquid from permeating the sheet of paper. The sulpho-cyanide salt alters the natural lemon-yellow color of the fluid to a deep scarlet, which becomes colorless, when the paper is exposed to light, and thus serves to enable the operator to determine when the printing is finished.

In the second coating, ether or other volatile liquids serve, on the one hand, to make the tannic acid or similar substances assume the form of paste, in which condition the coating operation is greatly facilitated, and adhesion after drying is perfected, while they inhibit, on the other hand, the chemical combination of the tannic acid with the ferric salts, thus preventing the production of blackish substances.

In the accompanying drawing the thin layer, 1, of tannic acid or similar substances is placed on the thin gelatine film, 2, made of the first coating of ferric salts, ammonium sulpho-cyanide, etc., in gelatine solution which is applied on a tenacious thin paper sheet, 3, well sized with alum-gelatine water.

Now in the actual practice, after the exposure to light the ferric salts lying under the black lines of the original transparent drawing from which the print is made will combine with the thin layer of the tannic acid when the paper is soaked in water, and in such a way black line duplicates are secured. In the exposed surface, the ferric salts are converted to ferrous salts which produce no

55

60

65

70

75

80

95

90

100

colored material in the presence of the tannic acid.

Ferric salt papers, hitherto prepared are of an inconspicuous lemon-yellow color, the observation of which, in measuring the degree of whitening when exposed to light, is a matter of great difficulty, while with my paper, it being colored a deep scarlet, the operator can easily determine the degree of exposure by the whitening. Some papers on the market use a special developing liquid after exposure to light to develop the black lines. This process, however, is somewhat complicated in operation, and the black lines printed are not satisfactory in color intensity and the finishing of the blank surface of the paper is not clear unless the printed paper is subjected to some bleaching chemicals which weaken the printed black lines. Others are made by pressing and rubbing the surface of the ferric salt coating with powder of the gallic acid. In this method the operation of pressing and rubbing the slippery surface of the paper as well as the degree of adhesion of the powder to the first coating may not be expected to be satisfactory as a matter of fact. Consequently, the black lines secured are not satisfactory and lack uniformity. In this process the sensitized paper can only be kept in its original condition for a short time after manufacturing, as the acidic and alkaline chemicals will gradually spoil the cellulose of the paper sheet, which loses its tenacity and becomes too frail to endure washing. Gelatine, that has the merit of absorbing chemicals to guard the cellulose of paper against spoiling, can not be used in this process. For, in case gelatine be a component of the coating, the gallic acid powder is not fixed on the gelatinous slippery surface.

In my process, the volatile pasty solution is applied on the gelatinous coating. Therefore, the operation is simple, easy, complete and even over the whole surface. And as the thin layer of the second coating adheres tightly to the first, the black lines thus revealed are clearly printed and retain intensity of color.

The manipulation of my paper is practically the same as when using ordinary blue-printing photo paper. The new paper is placed under the original transparent drawing in a frame and exposed to sunshine or an electric arc-light, and when those portions of the paper, over which black lines or spots of the original transparent drawing do not exist, have lost their original scarlet color and turn white, the exposed paper is taken off the frame and soaked in water. Then the parts left in scarlet lines or spots which have not been exposed to the light, turn black. The sheet is then placed on a smooth plate with the surface upward and washed with sponges soaked in water, and after being well sprinkled with water, the printed sheet is dried for actual use.

While I have shown and described the process which I now consider to be the best embodiment of the invention, I desire to have it understood that such changes may be made in the process when desired as are within the scope of the invention as claimed, and, accordingly, therefore do not wish to be limited to the details described herein.

Having now described my invention, what I claim as new, and desire to secure by Letters Patent, is:—

1. A sensitized photographic paper comprising paper having a coating of ferric salts and a superposed coating of tannic acid.

2. A sensitized photographic paper comprising paper having a coating of ferric salts and a soluble sulphocyanide, and a superposed coating of tannic acid.

3. A sensitized photographic paper comprising paper having a coating of ferric salts, a soluble sulphocyanide, tartaric acid and gelatine, and a superposed coating of tannic acid.

4. The process of making a sensitized photographic paper which comprises coating a paper with a solution of ferric salts containing a soluble sulphocyanide, drying the coated paper and then applying a solution of tannic acid in a volatile solvent thereto.

In testimony whereof I hereby affix my signature this 28th day of December, 1927.

RYO OMOTO.

100

105

110

115

120

125

130